

March 15, 1949.

W. B. CARDEN  
PROCESS OF PRODUCING VISCOSE  
RAYON YARNS AND FABRICS  
Filed Oct. 8, 1945

2,464,433

FIG. 1.

Viscose rayon treatment from  
individual filament stage.



FIG. 2.

Viscose rayon treatment of  
cut, staple or spun filament.



INVENTOR.  
William B. Carden.

BY *Alvans R. Powell*  
Lancaster, <sup>Av</sup> *Alvans R. Powell*

ATTORNEYS.

Patented Mar. 15, 1949

2,464,433

# UNITED STATES PATENT OFFICE

2,464,433

## PROCESS OF PRODUCING VISCOSE RAYON YARN AND FABRIC

William B. Carden, Beauport East, Quebec, Canada, assignor of one-half to Elizabeth M. Carden, Beauport East, Quebec, Canada

Application October 8, 1945, Serial No. 620,891

4 Claims. (Cl. 28—74)

1

This invention relates to the improved process or method of processing viscose rayon fabric to give it increased resistance to fatigue.

The primary object of this invention is the provision of an improved method of tire fabric formation wherein viscose rayon filaments are treated in such manner in the formation of the fabric used in rubber tires as to preserve the original strength of the filaments entering into the makeup of the strands of the fabric and to give the same added resistance to rupture or fatigue to which they are subjected by constant tire flexing under conditions of load and heat.

A further object of this invention is the provision of an improved imperviously sealed lubricated viscose rayon fabric.

A further object of this invention is the provision of an improved tire having incorporated therein multi-ply fabric layers which are extremely resistant to fatigue or breakdown.

Other objects and advantages of this invention will be apparent during the course of the following detailed description.

In the accompanying drawing, forming a part of this specification and wherein similar reference characters designate corresponding parts throughout the several views—

Figure 1 is a diagrammatic representation of processing or treating steps wherein viscose rayon treatment starts with an individual filament stage.

Figure 2 is a diagrammatic representation of steps in a process which includes the improved treatment of cut, staple or spur viscose filaments.

At the outset, I am familiar with prior art processing of rayon strands wherein oils and lubricants have been used on the filaments or strands to facilitate mechanical handling necessary for fabrication of the rayon yarn. The lubricant so used is removed by scouring or wiping in the finished fabric. I am also familiar with a process of treating cellulose acetate rayon yarn with a so-called lubricant which, if used in treating viscose rayon yarn, would defeat the purpose of rendering the fabric fatigue resistant. That is true because cellulose acetate rayon is made from material (cotton linters) fundamentally different from the material (wood pulp) of which viscose rayon yarn is fabricated. As a result, viscose rayon filaments (which make up the strands forming the fabric) have a greater affinity for moisture or absorption. I have found that the only satisfactory material usable as a lubricant in the process to be subsequently described, for treating viscose yarn, is a vegetable oil which is a non-penetrant and deposits merely a film of lubrication upon the filaments and between the filaments forming the strands in the finished cord or yarn. Therefore, my lubricant, preferably olive oil, is of a non-aqueous nature and this in-

5 sures the retention of the original strength of the filament and gives added resistance to fracture or fatigue in the fabric, wherever the fabric is used, such as in the case of a rubber tire where such fabric is subjected to continuous flexing under conditions of load and temperature which sometimes are unusual. The use of a non-aqueous lubricant prevents swelling and absorption, and thus there will be no weakening of the individual filaments or the yarns. In other words, they preserve their original tensile strength and the lubricant has no deleterious effect whatsoever. This remains in the filament throughout the life of the fabric because it is imperviously sealed in a coating of rubber or latex.

Referring to the diagrammatic processing steps outlined in Figure 1 of the drawing, the same are applicable to the treatment of viscose rayon where individual continuous filaments are used, 10 from the filament stage. While I do not wish to be limited to any particular weight or size of the yarn, the strands for tire manufacture are each formed of 480 filaments, 1100 denier. Thus, as shown in Figure 1, the step 10 consists of assembling 15 the continuous individual filaments in a strand. They are arranged parallel, and in step 11 they are loosely twisted together in about two or three turns or twists to the inch. The strands then pass through a bath of lubricant 20 at 11a; preferably a trough placed in back of the rolls in the twisting machine. The lubricant coats the individual filaments, since as above mentioned they are but loosely twisted. Thereafter, the lubricated strands are additionally 25 twisted at 12, preferably substantially 14 twists to the inch; the twist being in the same direction as previously provided in step 11. Thereafter in step 13 a plurality of the strands are placed together. With the weight and size of filaments 30 above specified the number of strands used in step 13 is preferably only two. They are then drawn through a lubricating bath 14 which thoroughly coats the individual strands of the multiple strand assembly, and thereafter at 15 these strands are additionally twisted, but in a direction opposite to the twists of the individual strands accomplished in steps 11 and 12. This twisting in reverse totals substantially 12 twists or turns to the inch.

40 Thereafter the yarns may be woven or otherwise formed into fabric. The fabric formation may vary, preferably a few filler threads per inch being incorporated if the fabric is of a type adapted to be used in the formation of rubber tires. After the fabric is formed it is entirely coated with some impervious flexible material such as rubber, rubbery latex or other plastic which may be applied in any of the usual ways, such as by frictioning. The fabric formation is 45 designated at 16 in Figure 1 of the drawing, and

the sealing coating step is indicated at 17. Thereafter there is a cutting step 18 wherein the fabric, if intended to be used for tire formation, is cut in strips on the bias. The cut fabric at 18, for tire formation, is then arranged in layers within the carcass of the tire.

As before mentioned the lubricant used in baths 11<sup>a</sup> and 14 is preferably olive oil or some non-aqueous vegetable lubricant. It must have an affinity for rubber or latex, or the coating used, to render the fabric impervious. The lubricant is not of a nature to bind the individual filaments together, as would be the case if some starch material or glue was used, as has sometimes been suggested for the purpose of giving yarn greater strength. With the lubricant suggested herein the filament does not lose its inherent flexibility. Thus, the finished yarn retains the resiliency necessary for the particular purpose defined herein, and obviously the processing of the viscose rayon through the sealing stage of the fabric will increase the resistance to friction and fatigue over rayon fabric which is not treated with a lubricant under the conditions specified.

It is also a purpose of this invention to process viscose rayon fabric formed of cut, staple or spun filaments. Thus, referring to Figure 2 in the initial processing step 25, the staple or spun filaments are tightly twisted so as to hold their short lengths and form a thread. Four or five of these threads are then assembled in a step 26 and subsequently at 27 pass through a lubricating bath containing a lubricant such as above mentioned (olive oil). This completely films the threads with oil. At 28 these assembled threads are then twisted into strands; the twisting being reversed or opposed to the twisting of the individual threads at 25. This enables the oil or lubricant to contact and coat the individual filaments; that is, penetrate between the cut filaments. At 29 two of the strands arranged at 28 are assembled, although more may be used if desired, and subsequently they pass through a lubricant bath 30 similar to the bath 14. The process from there on, as indicated in the drawing, follows the process for the viscose rayon individual filament fabric as shown in Figure 1.

In addition to the advantages above enumerated, the lubrication treatment to which the rayon is subjected with the non-aqueous lubricant used naturally renders this fabric less impervious to moisture and humidity than untreated fabric or yarn.

Baggy fabric or sagging sections across the width of the fabric is a constant source of annoyance and waste after it is received at a rubber mill for processing. This will be eliminated in my fabric.

Manufacturers using rayon fabric ordinarily place the rayon cord, which is wound on spools or cones, through an electric heater or drier to set the twist, so that the cord will be better balanced and less apt to kink. Thereby handling is facilitated in the beaming and weaving operations. With my improved lubricated yarn the cords are naturally set and the heating and drying processing will not be necessary.

Lubrication of the yarns will also lubricate the rings on the twisting mechanism and thus eliminate the necessity for supplying separate lubricant therefor.

While I prefer to use olive oil as the lubricant, cottonseed oil, soya bean oil and peanut oil or

any vegetable oil not deleterious to the filament or rayon yarn may be used.

Various changes in the steps of the processes and methods herein designated may be made to the above description, and the fabric may be incorporated in various ways and applied to various uses without departing from the spirit of this invention and the scope of the claims.

I claim:

1. The process of producing viscose rayon yarn which consists in an initial assembly of viscose rayon filaments, passing the same through a lubricating bath of a non-aqueous vegetable oil in such manner as to individually coat the filaments with the lubricant, subsequently twisting said filaments into strands without interfering with the individual lubricating film coating of the filaments, subsequently providing a plurality of said strands and coating them by passing them through a lubricating bath of a non-aqueous vegetable oil, and subsequently twisting said assembled strands into yarn without interfering with the individual film coating of the filaments and strands.

2. A process of producing viscose rayon yarn which consists in assembling individual viscose rayon filaments of a desired number to provide a strand, very loosely twisting the filaments, subsequently passing said filaments through a lubricating bath of non-penetrant oil to coat them without impregnation, subsequently additionally twisting said filaments into strand formation, subsequently placing a number of said strands together and coating them by passing them through a lubricating bath of a non-penetrant oil, and subsequently oppositely twisting said assembled strands to form yarn.

3. A process of manufacturing viscose rayon yarn which consists in taking a number of spun viscose rayon twisted threads, assembling a plurality of said twisted threads and passing them through a lubricating bath of vegetable oil, subsequently twisting the thus assembled threads in a direction opposite to the filament twist of the threads, thereafter providing a multiple strand assembly of said strands as previously twisted and then passing them through a filament coating lubricating bath of vegetable oil, and then oppositely twisting said assembled strands into yarn formation.

4. The process of producing viscose rayon fabric which consists in film coating viscose thread strands with a non-penetrant lubricating oil, providing of said strands a multiple strand assembly, film lubricating said assembly with a non-penetrant oil, twisting the strands to form yarn, manipulating the yarn to provide fabric, and entirely coating said fabric with flexible impervious rubber to prevent lubricant dissipation.

WILLIAM B. CARDEN.

#### REFERENCES CITED

The following references are of record in the file of this patent:

#### UNITED STATES PATENTS

| Number    | Name           | Date          |
|-----------|----------------|---------------|
| 1,356,920 | Jury           | Oct. 26, 1920 |
| 2,058,778 | Dinsmore       | Oct. 27, 1936 |
| 2,089,188 | Dreyfus et al. | Aug. 10, 1937 |
| 2,126,314 | Dickey         | Aug. 9, 1938  |
| 2,132,492 | Parker         | Oct. 11, 1938 |
| 2,319,077 | McNally et al. | May 11, 1943  |
| 2,364,135 | Finlayson      | Dec. 5, 1944  |